

## UNITED STATES PATENT OFFICE

2,079,058

MACHINEABLE STEEL AND ARTICLES  
FORMED THEREFROMLouis H. Winkler, Bethlehem, Pa., assignor to  
Bethlehem Steel Company, a corporation of  
PennsylvaniaNo Drawing. Application February 20, 1934,  
Serial No. 712,138

6 Claims. (Cl. 75—123)

My invention relates to bodies, such as screws, which involve as steps of their manufacture, upsetting or cold forming, and machining operations. My invention comprises articles of manufacture, such as screws, of rimmed steels containing percentages of sulphur sufficiently great to render them easily machineable. This invention further comprises such steels themselves.

Relatively high sulphur contents have been used for some time in machining steels, particularly in screw stock. Rimmed steels of low sulphur content have been long well known and widely used for various purposes. I have discovered that sulphur in large enough amounts to confer easy machineability, particularly for threading operations, may be added to rimmed steel with beneficial results in the manufacture of such articles as screws. Such steels have excellent upsetting and cold forming properties and therefore they may be readily headed as, for example, in screw manufacture.

When, prior to my invention, relatively high contents of sulphur were used for conferring ready machineability the steels thus produced frequently had surface imperfections, such as seams, which caused difficulty in upsetting and cold forming operations and giving at times more or less unsatisfactory products. To prevent or nullify these imperfections additions of some deoxidant, aluminum for example, have been made, but the resulting steels, as a consequence of these additions, frequently offered difficulties in machining. By my invention these obstacles to upsetting, cold forming and machining are overcome. Because of the rimming of the steel the surface or "skin" is substantially free from the imperfections which have rendered upsetting operations difficult and uncertain and, rather surprisingly, the surface condition, thus produced by rimming, does not interfere with the action of the sulphur in facilitating the machining operations. Obviously the employment of this practice makes unnecessary the use of any considerable quantity of deoxidants as heretofore and avoids the deleterious effect of such additions on the machining qualities.

I employ steels having carbon contents up to .25%, manganese up to .60%, and silicon preferably not exceeding .03%. The usual methods for making rimmed steel are employed. Aluminum additions are preferably avoided. Sulphur is

added to the steel in the ladle after it has left the steel producing furnace, sufficient of this element being added to give a sulphur content in the finished steel of from .07% to .25%. Sulphur may be added in any desired form, as for example 5 as stick sulphur or as pyrites.

For wood screw stock I employ rimmed steel preferably containing carbon from .10% to .20%, and sulphur from .10% to .16%, although I have obtained satisfactory results with sulphur as low 10 as .08% and as high as .18%. Such steels are readily adapted to upsetting operations and they thread easily giving accurate threads free from appreciable imperfections.

Rimmed steels containing carbon .06% to .12% 15 and sulphur .07% to .20% have given good results in the manufacture of machine screws, the results being especially good with carbon .06% to .10% and sulphur .08% to .12%. In making machine screws with these steels standard methods of manufacture may be employed. The properties due to the rimming of the steel facilitate the forming operations such as upsetting and thread rolling without interfering with the effects of the sulphur in aiding the machining operations 20 such as shaving and slotting of the heads.

Having thus described my invention what I claim as new and desire to secure by Letters Patent is:

1. Screw stock of rimmed steel containing carbon up to .25%, and sulphur .07% to .25% and the balance consisting substantially of iron. 30
2. Wood screw stock of rimmed steel containing carbon .10% to .20% and sulphur .08% to .18% and the balance consisting substantially of 35 iron.
3. Machine screw stock of rimmed steel containing carbon .06% to .10% and sulphur .07% to .14% and the balance consisting substantially of iron. 40
4. A wood screw of rimmed steel containing carbon .10% to .20% and sulphur .07% to .25% and the balance consisting substantially of iron. 45
5. A machine screw of rimmed steel containing carbon up to .12% and sulphur .07% to .12% and the balance consisting substantially of iron. 50
6. A machine screw of rimmed steel containing carbon up to .12% and sulphur .07% to .25% and the balance consisting substantially of iron. 50

LOUIS H. WINKLER.